

A. R. ROWE,  
APPARATUS AND METHOD FOR CASTING METAL PRODUCTS,  
APPLICATION FILED MAY 3, 1921.

1,399,798.

Patented Dec. 13, 1921.

2 SHEETS—SHEET 1.



Inventor  
Andrew R. Rowe

By

T. M. Duthie & Son

Attorney

A. R. ROWE.

APPARATUS AND METHOD FOR CASTING METAL PRODUCTS.

APPLICATION FILED MAY 3, 1921.

1,399,798.

Patented Dec. 13, 1921.

2 SHEETS—SHEET 2.



Inventor  
Andrew R. Rowe

Matthews

By

Attorney

# UNITED STATES PATENT OFFICE.

ANDREW R. ROWE, OF PORTSMOUTH, OHIO.

## APPARATUS AND METHOD FOR CASTING METAL PRODUCTS.

1,399,798.

Specification of Letters Patent.

Patented Dec. 13, 1921.

Application filed May 3, 1921. Serial No. 466,564.

To all whom it may concern:

Be it known that I, ANDREW R. ROWE, a citizen of the United States, residing at 1908 21st street, Portsmouth, in the county 5 of Scioto and State of Ohio, have invented certain new and useful Improvements in Apparatus and Methods for Casting Metal Products, of which the following is a specification.

10 This invention relates to improvements in devices for casting iron and steel ingots and other metal products and the primary object of the invention is to furnish a novel molding device or mold attachment which 15 will eliminate defects now found in molding molten metals.

In the manufacture of iron and steel and other metal products, especially high carbon steel, great difficulties are encountered 20 in casting solid compact ingots due to the formation of blow-holes and "pipe", which are formed in the process of pouring and during the period of solidification.

Blow-holes or bubbles caused by trapped 25 gases in the cast metal, it is found, do not always weld during subsequent rolling of the metal.

When the metal is first poured in the mold, the mold being cold, the metal freezes 30 to the mold. In other words, the ingot due to the difference in temperature between the metal and the mold, shrinks away from the center toward the sides of the mold. When the pouring of the ingot is finished, 35 the top freezes over, the metal shrinking toward the sides causing a sinkhead or gas pocket due to the fact that the metal freezing on top does not allow sufficient metal to fill the shrinkage cavity formed during the period of solidification.

In the ordinary method of pouring ingots, the metal is discharged from a ladle. The ladle may contain as high as one hundred tons of metal, the ladle nozzle usually being from two to three inches in diameter through which the metal is poured into the mold. Due to the quantity of metal in the ladle, it is evident that there is a heavy head pressure on the metal issuing from the ladle nozzle, and as the metal rises in the mold, this stream, due to the heavy head

pressure, forces itself to a considerable depth into the metal already poured into the mold, and this causes the slag and impurities which may come to the surface to be forced down again into the metal in the mold, and gases in the form of blow-holes forced deep into the metal cannot rise to the surface readily until the stream from the ladle is shut off. Some of the blow-holes 55 or gases are forced too deep into the metal to again rise to the surface, and the top freezing over quickly traps the gases within the metal and prevents their escape. 60

There are known methods in practice 65 which lessen the liability of blow-holes, in the metal ingot, and to a certain extent eliminate "pipe", but they are usually such that they entail great overhead expense and retard production. 70

The method and apparatus forming the subject-matter of the present invention may be used with very little added expense over the common or ordinary method and apparatus used in pouring metals and without 75 retarding production.

The invention will be described in detail in connection with the accompanying drawings, in which:

Figure 1 is a detail sectional view of an 80 ordinary mold illustrating the manner in which the jet of metal from the ladle nozzle penetrates the metal in the mold and causes blow-holes, "pipe", sinkheads or gas pockets and the like.

Fig. 2 is a similar view of a mold with my improved attachment applied thereto and illustrating the manner in which the heavy head pressure in the ladle is counteracted so that relatively small jets of metal 85 will fall into the mold without an excess of head pressure.

Fig. 3 is a similar view illustrating a mold provided with my attachment and showing the float valve with which my attachment is equipped, raised by the metal which has been deposited in the mold.

Fig. 4 is a sectional view of a mold with a modified form of my attachment applied thereto and showing the operation of the 100 same before the mold has been entirely filled.

Fig. 5 is a similar view of the modification but showing the floating valve raised by the metal in the mold.

Fig. 6 is a top plan view of the form of attachment shown in Figs. 2 and 3.

Fig. 7 is a similar view of the modified form of attachment shown in Figs. 4 and 5.

Referring to Fig. 1, 1 designates an ordinary mold into which molten metal is poured from the ladle nozzle 2. This view illustrates the apparatus and method now in use for molding or casting ingots and it will be seen that a relatively large jet or stream 3 with considerable head pressure behind it flows downwardly into the mold 1. Owing to the head pressure on the jet 3 said jet will penetrate to a considerable distance below the surface of the metal in the mold and will cause the blow-holes or trapped gases 4 to be forced beneath the surface of the metal and to remain in the position to which they are forced. In addition to this the difference in temperature between the molten metal and the mold 1 will cause the top of the metal in the mold to freeze or quickly solidify when the pouring is complete and this will cause a sinkhead or gas pocket 5 to be formed at the upper end of the cast ingot.

It is to eliminate these defects in the known molding device and method that I have provided my improvements which will now be described:

Referring to Figs. 2, 3 and 6, 1<sup>a</sup> designates the mold to which I attach a tubular reservoir 6 which is provided with an external shoulder 7 designed to rest on the upper edge of the mold, and a tubular extension 8 which projects into the mold. At the lower end of the tubular body 1 I provide an inwardly extending annular flange 9 which supports a float valve 10 having a plurality of apertures 11. If desired, the tubular body may be surrounded by a reinforcing metal band or jacket 12 which in a measure, protects the body 6 that is preferably formed of refractory material.

The body 6 is also preferably provided with gas vents 13 which extend from the top to the bottom of the body and function to release gases from the mold as the metal is poured into the same.

With this form of the invention the metal from the ladle will be poured through the nozzle 2<sup>a</sup> and will enter the reservoir where a portion of the same will accumulate. This small body 14 of the metal within the reservoir will flow through the apertures 11 in the valve 10 and these small streams will not penetrate into the metal in the mold to any great extent, and the gases rising from the metal in the mold will not be interfered with by these small streams. Hence no blow-holes or "pipe" will be left in the cast ingot.

When the metal in the mold rises to a point 65 where it engages the float valve 10 it will lift this float valve as shown in Fig. 3, and the metal which is cast in the mold will be free of blow-holes and "pipe."

The embodiment illustrated in Figs. 4, 5 70 and 7 carries out the same result as the device shown in Figs. 2, 3 and 6, but in this instance the mold 1<sup>b</sup> is preferably provided near its upper end with an internal annular shoulder 1<sup>c</sup> on which rests the lower end of 75 the reservoir 6<sup>a</sup>. This reservoir is preferably provided with a solid or imperforate float valve 10<sup>a</sup> which normally engages a seat provided in an inwardly extending annular ledge or flange 10<sup>b</sup>. In this form instead of discharging the metal through the valve, I discharge the same through apertures or ports 11<sup>a</sup> provided in the ledge 10<sup>b</sup>. Gas vents 13<sup>a</sup> are also provided in this construction. The operation of the modified 80 form of the invention is the same as that described in connection with the other form with the exception that the metal flows from the reservoir 6<sup>a</sup> through ports provided in the reservoir instead of in the valve. 90

The reservoir and float valve are preferably made of some refractory material, such as fire-clay, brick, or material that is heated quickly and does not rob the metal of but very little of its original heat. 95

The size of the holes in the reservoir or floating valve are to be determined by the size of the pouring nozzle of the ladle.

Reverting again to the operation of the device, the metal is poured from the ladle 100 into the reservoir and it then drains through the holes in the reservoir or floating valve into the mold proper, this eliminating the heavy head pressure from penetrating or forcing the metal into the body of metal contained in the mold, confining the same to the reservoir and allowing the metal to flow through the holes without any penetrating effect upon the metal as it rises in the mold. I preferably provide the apertures in the 105 reservoir or floating valve at points off the center of the mold, so that the streams draining down allows the center of the ingot or metal, which is the hottest part of the metal, to freely discharge gases or air and thus 110 form a more solid and compact ingot. It may be readily seen that by pouring the metal into the reservoir that a great portion of the gases escape from the metal in the reservoir before the metal enters the mold, and the elimination of the heavy head pressure prevents blow-holes in the form of trapped gases from being forced down into the metal of the mold proper. Also, during the process of pouring into the reservoir, the walls 115 of the reservoir become heated to such a high degree that the metal which is last poured into the reservoir, when the mold and reser- 120 125

voir are both filled, will lose none of its original heat through contact with the walls of the reservoir and when the stream is shut off in the ladle the floating valve which is 5 lighter than the metal, and being a foreign substance from the metal, will rise to the top of the reservoir as before described. The reservoir, which has become highly heated during the pouring of the metal, will retain 10 the heat on the top or upper portion of the ingot for a longer period than has so far been obtained without using any expensive fuels or gases.

By eliminating the heavy head pressure 15 back of the stream of metal and confining the same to the reservoir the mold proper is allowed to fill without any danger of splash which oftentimes freezes to the mold and does not weld to the ingot as is desired, 20 leaving a scabby surface on the ingot which is objectionable.

The mold proper being fed by the small streams or jets with little or no head pressure allows the metal to rise in the mold 25 evenly and at the same time gives the gases and impurities a better chance to reach the surface. When the mold and reservoir are filled and solidification starts, the metal in the upper portion of the reservoir will 30 readily supply the shrinkage cavity and confine the sinkhead to the reservoir, thus providing a compact solid ingot.

The floating valve which rests on the lugs of the reservoir may be square, oblong, 35 round or any shape desired. The valve may also be flat, arched or convexed and the edge which fits in the valve seat should be tapered and smooth and the valve seat should also be smooth.

40 When the ingot has cooled in the mold, the mold is stripped from the same by the ordinary method now in use, the reservoir being eliminated during the process of stripping the mold from the ingot.

45 It will also be noted that my attachment may be employed with an ordinary mold without altering the same or by making the simple alteration of the internal shoulder 1° as shown in Figs. 4, 5 and 7.

50 Most plants or concerns that make high carbon ingots in particular, are obliged to use a separate method or different molds, for instance, large end of mold inverted or mold inverted after the pouring, movable walls, 55 and methods for liquid forging, vibrators or apparatus for stirring and various other methods which necessitate heavy expenditures, changes in stripping apparatus resulting in loss of time and retarding production.

60 With the present method, the same molds may be used for soft steel or high carbon steel without loss of time or without retarding production and with increased efficiency in regard to production or per cent. of steel 65 free from "pipe" per ingot.

From the foregoing I believe that the construction, operation and advantages of my invention may be readily appreciated by those skilled in the art, and I am aware that various changes may be made in the constructions illustrated and described without departing from the spirit of the invention as expressed in the following claims.

What I claim and desire to secure by Letters-Patent is:

1. A method of depositing materials in a mold which consists in providing an open top body for the material in the upper end of the mold, discharging material into said body in a relatively large jet, discharging material from the body into the mold in relatively small streams and conducting the air from the mold around the exterior of the material in the body.

2. A method of depositing molten metal 85 in molds which consists in discharging a relatively large stream of molten metal into an open top body intercepting this stream of metal in the body before it reaches the mold and forming a pool of the metal, discharging the metal from said pool into the mold in relatively small streams and conducting the air from the mold around the exterior of the metal pool.

3. A method as set forth in claim 2 in 95 which gases are discharged from the mold during the depositing of the metal in the mold by the small streams.

4. A method as set forth in claim 2 in 100 which the points at which the relatively small streams enter the mold are elevated near the completion of the filling of the mold.

5. A method as set forth in claim 2 in 105 which the relatively small streams enter the mold at points spaced from the axis of the mold.

6. An apparatus for molding metal comprising a mold, a reservoir member provided at the upper end of said mold, a float valve 110 member coöperating with the reservoir member, and apertures provided in one of said members for discharging metal from the reservoir into said mold.

7. An apparatus of the kind defined by 115 claim 6 in which the reservoir is provided with gas vents to permit the escape of gases from the mold.

8. An apparatus of the kind defined by 120 claim 6 in which the reservoir and valve are formed of refractory material.

9. An apparatus of the kind defined by 125 claim 6 in which the reservoir is provided with a metal jacket.

10. An apparatus of the kind defined by 125 claim 6 in which the lower end of the reservoir projects into the upper end of the mold.

11. A pouring attachment for molds comprising a reservoir provided at its lower end with a floating valve, apertures provided 130

- 4.
- in the reservoir for discharging metal from the same into a mold, and gas vents formed in the reservoir for permitting the discharge of gases from the mold.
5. 12. A pouring attachment for use with a metal mold comprising a tubular reservoir member provided at its lower end with an inwardly extending annular flange, a float valve member normally resting on said flange, and apertures provided in one of
- said members for discharging metal from the reservoir into a mold.
13. An attachment of the kind defined by claim 12 in which the reservoir is provided with gas vents. 15
14. An attachment of the kind defined by claim 12 in which the reservoir member is surrounded by a metal jacket.

In testimony whereof I affix my signature.  
ANDREW R. ROWE.